# EUROPEAN PATENT APPLICATION

(11) **EP 0 100 659 A1**
(43) Date of publication of application: **15.02.1984**
(21) Application number: 83304386.2
(22) Date of filing: 28.07.1983
(51) Int. Cl.: C25B 11/04, C25B 1/46, C23C 4/18, C23F 1/36

(54) **Process for making Raney nickel coated cathode, and product thereof**

(30) Priority: 30.07.1982 US 403306
(71) Applicant: E.I. DU PONT DE NEMOURS AND COMPANY, Wilmington Delaware 19898 (US)
(72) Inventor: Bhedwar, Homi Cawas, Hockessin Delaware 19707 (US)
(74) Representative: Myerscough, Philip Boyd (GB)

(57) **Abstract**

Raney-nickel coated cathodes are made by plasma spraying a nickel/aluminum composition containing 56 to 59% by wt. nickel onto an electrically conductive cathode substrate, and activating the coated substance by leaching aluminum from the coating with caustic. The activated cathode is especially useful in chloralkali processes, as it operates at low hydrogen overvoltage, and is durable against spalling and flaking.

## Description

### BACKGROUND OF THE INVENTION

This invention relates to a process for making an improved low hydrogen overvoltage cathode of the Raney nickel type for use in chloralkali electrolysis, and to the cathode so made.

Cathodes of the Raney nickel type are known. in the art, e.g., U.S. 4,116,804, U.S. 4,169,025 and U.S. 4,251,344. However, Raney nickel coated cathodes of the prior art, while initially exhibiting good performance characteristics, suffer certain defects. Such Raney nickel coating on the cathode substrate has been of low durability, i.e., easily mechanically damaged and lost even by, e.g., water jets. For example, when such a cathode is used in a diaphragm-type chloralkali cell wherein an asbestos diaphragm is deposited directly onto the cathode surface, such diaphragm gradually loses its permeability due to clogging of the pores, usually after about 9 to 15 months, and must be removed and replaced; removal is ordinarily accomplished by spraying with jets of water, and during such spraying, the jets of water have caused loss of some of the Raney nickel by flaking or spalling. When the replacement diaphragm is deposited and baked, ordinarily at 355°C in air for 4 hours, some deactivation of the Raney nickel coating by oxidation occurs. This progressive spalling and deactivation of Raney nickel after multiple washes and bakes is responsible for a progressive loss of the voltage benefit provided by the Raney nickel, i.e., the operating voltage of the cathode progressively increases and approaches the operating voltage of the cathode substrate.

Accordingly, it is a principal object of this invention to provide an improved Raney nickel coated cathode having a more durable Raney nickel surface than those previously known, and a process for making same.

Other objects will appear hereinafter.

### SUMMARY OF THE INVENTION

Briefly, according to the present invention, there is provided a process for making a durable, low-hydrogen-overvoltage cathode for chloralkali use which comprises applying a nickel/aluminum alloy composition containing 56 to 59 % by weight of nickel onto a suitable cathode substrate by plasma spraying, followed by leaching with caustic to remove aluminum.

More specifically, there is provided in accordance with the invention a process for making a low-hydrogen-overvoltage cathode for a chloralkali cell which comprises
(a) plasma spraying a coating of a nickel/aluminum alloy composition containing 56 to 59% by wt. nickel onto a foraminous substrate of iron, ferrous alloy, nickel or nickel alloy, and
(b) leaching aluminum from said coating by contacting the article prepared in step (a) with a caustic solution.

There are also provided in accordance with the invention a Raney nickel coated cathode made by said process, a chloralkali cell containing said cathode, and a process for electrolysis of an alkali metal chloride in said cell.

### DETAILED DESCRIPTION OF THE INVENTION

In the present invention a selected nickel/aluminum alloy composition is applied to an electrically conductive cathode substrate by plasma spraying.

It is a requirement of the present invention that the nickel/aluminum alloy composition employed for deposition on the cathode substrate contain about 56 to 59% by wt. nickel. Nickel/aluminum alloys in this composition range contain the intermetallic compound Ni₂A1₃ as the predominant phase, but also contain minor amounts of NiAl and NiAl₃, the exact amounts of these varying with the specific overall composition. Preferably, the nickel/aluminum alloy composition contains 56.5 to 57.5% by wt. nickel, most preferably substantially 57% by wt. nickel.

The nickel/aluminum alloy is suitably employed in the form of particles or granules, preferably 36 to 90 microns (165 to 400 mesh) in size, more preferably 36 to 53 microns (270 to 400 mesh) in size.

The electrically conductive cathode substrate can have various configurations, e.g., flat, tubular, fingers, etc., but in any case should be foraminous, e.g., woven wire screen, expanded sheet metal or punched sheet metal. Iron, ferrous alloys such as mild steel and stainless steel, nickel and nickel alloys are particularly suitable materials for this substrate.

It is another requirement of the present invention that the nickel/aluminum alloy composition be deposited on the cathode substrate with the use of plasma spraying, also termed plasma arc spraying. Plasma spraying is a known technique for depositing metal particles onto a substrate. Briefly, streams of a gas and the metal particles are separately fed to a spray nozzle, (torch), and there is an electrical power input to the gas stream which ionizes the gas; recombination of the positive ions and electrons in the gas stream after mixing with the metal particles releases energy which heats and partially melts the metal particles, and the partially melted metal particles adhere to the substrate on contact with it. Various gases, including nitrogen and argon, are suitable gases for this purpose. Argon is a preferred gas. The power input need only be sufficient to partially melt the metal particles, e.g. 20 to 30 kilowatts in apparatus of ordinary size.

In most cases it is preferred to coat the fabricated cathode component rather than to coat the foraminous sheet material used to fabricate the cathode, because welding and other assembly techniques are more easily accomplished with the substrate in the uncoated condition. Also, it is best to clean the surface of the substrate before coating, as by sandblasting, or blasting with other grit such as alumina.

The cathodes of this invention can be either one-side or two-side coated. However if only one side is coated it is preferred to coat the side'which will face the membrane or diaphragm in order to obtain the maximum reduction in cell voltage.

Thickness of the nickel/aluminum alloy coating applied to the cathode substrate of about 13 to 508 microns (0.5 to 20 mils) is suitable, and is preferably about 127 to 254 microns (5 to 10 mils).

Following deposition of the nickel/aluminum alloy composition on the substrate, the Raney nickel surface is developed by contacting the coated article with any strong base such as a caustic solution so as to leach aluminum from the coating. The concentration of the caustic is not critical; aqueous caustic solution containing 5 to 15% by wt. NaOH is suitable for this purpose, and 5 hours to 1 day is adequate time for the leaching. A 10% by wt. aqueous caustic solution for 16 hours is typical. Similarly, the temperature for leaching is not critical; temperatures from room temperature up to the boilihg point of the caustic solution are suitable. For coatings of indicated thickness, about 70 to 90% of the aluminum will ordinarily be removed during such leaching; some aluminum appears to remain even after, much longer leaching time, but is believed not to be deleterious to performance of the resulting cathode. This leaching step is also referred to as activation, and can be carried out prior to or after assembly of the cell. The Raney nickel cathode so made, if permitted to dry, heats up upon contact with air, due to the pyrophoric character of Raney nickel.

The Raney nickel coated cathode so made not only exhibits low hydrogen overvoltage, but the coating has improved durability against flaking and spalling, as is shown hereinbelow in Example 9 and Comparative Examples B, C and D. As shown therein, the nickel/aluminum alloy composition applied as the coating in the process of the present invention provides an activated Raney nickel cathode surface which unexpectedly is much more resistant against spalling and flaking than those derived from alloys which contain 55% by wt. nickel or less, which spall at a commercially unacceptable rate. Also as shown therein, although all the compositions tested initially showed good reductions in hydrogen overvoltage, the improvement in hydrogen overvoltage unexpectedly was maintained at a higher level following wash/bake cycles in the case of the nickel/aluminum alloy composition applied as the coating in the process of the present invention than did those containing lesser (55% by wt. nickel and lower) and greater (62% by wt. nickel) amounts of nickel.

The cathode made by the process herein can be used as the cathode in known types of electrochemical cells which comprise a cathode compartment; a cathode disposed within said cathode compartment, an anode compartment, an anode disposed within said anode compartment, and a separator disposed between the anode and cathode compartments. It is especially useful in chloralkali cells of such description. The separator can be, e.g., a liquid permeable diaphragm; such diaphragm can be fabricated of, e.g., asbestos fibers or perfluorinated polymer fibers. The separator can alternatively be a membrane, e.g., of highly fluorinated or perfluorinated ion-exchange polymer; membrane of such polymer containing sulfonate and/or carboxylate groups is now well known in the chloralkali art, e.g., U.S. 4,192,725, U.S. 4,065,366 and U.S. 4,178,218. As is now known in this art, such membrane cells can be operated in both narrow gap (1-3 mm spacing from anode to cathode) and zero gap (both electrodes in contact with the membrane) configurations.

In a chloralkali process for electrolysis of an alkali metal chloride such as sodium chloride in such a cell, an aqueous alkali metal chloride solution is introduced into the anode compartment, an electric current is passed through the cell, an aqueous alkali metal hydroxide solution is removed from the cathode compartment and chlorine is removed from the anode compartment. In a membrane cell, water (or dilute alkali metal hydroxide at startup) is generally introduced into the cathode compartment, and spent alkali metal chloride solution is removed from the anode compartment. In a diaphragm cell,all of the unreacted alkali metal chloride solution percolates through the diaphragm into the cathode compartment, and is removed along with the product caustic.

The present invention has numerous advantages when compared to the prior art. These include (1) high resistance to flaking, spalling and mechanical damage of the activated coating; (2) resistance to oxidizing atmospheres, such as heating in air, e.g., during baking of a diaphragm thereon; (3) low hydrogen overvoltage compared to mild steel cathodes and Ni cathodes; (4) good tolerance to moderate amounts of contamination by iron overplating; (5) a variety of substrates including mild steel, stainless steel and nickel can be used; (6) low cost and convenient application to preconstructed cathode components; and (7) the substrate is rarely heated above 200°C, so that warping is minimal.

To further illustrate the innovative aspects of the present invention, the following examples are provided.

In the examples, abbreviations are used as follows:
PTFE refers to polytetrafluoroethylene;
TFE/EVE refers to a copolymer of tetrafluoroethylene and methyl perfluoro(4,7-dioxa-5-methyl-8-nonenoate) ;
TFE/PSEPVE refers to a copolymer of tetrafluoroethylene and perfluoro(3,6-dioxa-4-methyl-7-octenesulfonyl fluoride);
EW refers to equivalent weight.

### EXAMPLES

### Example 1

A commercial cathode screen made of 0.23 cm (0.092 inch) diameter steel wire spaced on 0.42 cm centers (6 mesh) was sandblasted, and then plasma arc coated on one side with a 178-203 micron (7-8 mil) thick coating of a nickel aluminide alloy whose composition was nominally 57% Ni, 43% Al; particle size range was 100% smaller than 90 microns (i.e., through 165 mesh) to 30% smaller than 42 microns (i.e., through 325 mesh). Spraying conditions were:
.Metco Type 7 MC (TMB) Torch-707 Nozzle
Metco 3MP Dual Power Feeders.
Torch Gas - 2.1 m³/hr (75 ft³/hr) nitrogen Volts - 60
Amperes - 425
Kilowatts - 27.3
No. of Passes - 5.

The screen surface was cooled with compressed air jets.

A sample portion of the screen was cut out, and a 7.62 cm (3 inch) diameter circular section cut from the sample. The circle was welded into a stainless steel cathode holder such that the coated side would face toward the anode in the subsequently assembled cell, leached in 10% caustic, and a PTFE fiber-asbestos diaphragm (TAB Diamond Shamrock composition) was deposited on the Raney nickel coated surface of the screen and baked. Performance of this cathode was as follows, with typical steel cathode performance given for comparison.

### Example 2

A cathode finger from a Diamond Shamrock MDC-55 cathode assembly was sprayed on one side with nickel aluminide of the same composition as in Example 1. Before the finger was sprayed, it was degreased and -sandblasted. Spraying conditions were:
Metco Type 7 MC (TMB) Torch-707 Nozzle
Metco 3MP Dual Power Feeders
Torch Gas - 2.1 m³/hr (75 ft³/hr) nitrogen Volts - 62
Amperes - 450
Kilowatts - 27.9
No. of Passes - 4.'

The screen surface was cooled with an air blast.

A sample was cut from this screen, leached in 10% caustic, coated with a TAB diaphragm directly on the Raney nickel coated surface, and tested in a 7.62 (3-inch) diameter diaphragm cell with the Raney nickel coated surface facing the anode. Performance of the coated sample at two different current densities was:

The advantage for the cathode of Example 2 vs. the steel cathode shown for comparison in Example 1 was 270 mV.

### Example 3

The fingers for three Diamond Shamrock MDC-55 cathode assemblies (cathode cans) were plasma sprayed with nickel aluminide of the same composition as in Example 1 under the conditions outlined under Example 2, only on the sides of the fingers which were subsequently coated with the diaphragm coating and which would face toward the anode. Each can was then leached for about 16 hours in cold 10% caustic solution. The cans were then washed, and a Diamond Shamrock TAB diaphragm deposited and baked on each. Each can was assembled into a chloralkali cell and operated in a cell line. All the cans performed similarly. Performance compared to steel was:

### Example 4

Samples of Type 304 stainless steel screen of 0.18 cm (0.072 inch) diameter wire spaced on 0.42 cm centers (6 mesh) were welded into stainless steel cathode rings and sprayed with a 0.015 cm (6-mil) thick coating of nickel aluminide of the same composition as in Example 1, only on that side to which the diaphragm coating was subsequently applied and which would face toward the anode in the subsequently assembled cell. The coating was leached with 10% caustic. A TAB diaphragm was deposited and baked onto the screens and the cathode assembly operated in a 7.62 cm (three-inch) cell. After initial operation, the diaphragms were removed, new diaphragms installed, and a second run made.

Data are:

### Example 5 - Preparation of a cathode for evaluation in a narrow gap membrane cell.

A cathode for a laboratory membrane cell was prepared by cutting out a 7.62 cm (3-inch) diameter disk of a flattene.d expanded metal having dimensions of 2.54 cm LWD (long way diamond) x 0.635 cm SWD (short way diamond) x 0.16 cm strand width x 0.12 cm thick of a type 200 nickel. A length of 0.635 cm nickel tubing was welded to the center of the disk to serve as a current conductor.

A coating of an alloy of 57% + 0.5% by wt. Ni and 43% + 0.5% by wt. Al was applied to both sides of this cathode by plasma spraying. The alloy was in the form of a fine powder having a particle size of 42 to 110 microns (i.e., between 140 mesh and 325 mesh). Conditions of application were as follows.

Power - 40 V and 580 A (23.2 kw) Arc Gas - 2.63 m³/hr (93 CFH) argon at 3.448 x 10⁵ Pa (50 psi) 10.16 cm (4 inch) TTWD (torch to work piece distance)

The coating thickness was 203 microns (8 mils) on both sides of the expanded metal. The coating was activated by immersing the cathode in a solution of 10% NaOH at room temperature for 16 hours. The cathode was then water rinsed and kept wet-until installed in a cell.

### Example 6 - Performance of a two-side coated cathode for evaluation in a finite gap membrane cell.

The cathode of Example 5 was mounted in a small cell having an active area of 45 cm², together with a reinforced fluorinated ion exchange membrane and a dimensionally stable anode. The membrane comprised a 38 micron (1.5 mil) layer of TFE/EVE having an equivalent weight of 1080; a 100 micron (4 mil) layer of TFE/PSEPVE having an equivalent weight of 1100, a layer of fabric having both PTFE filaments and polyethylene terephthalate filaments, and a 25 micron (1 mil) layer of TFE/PSEPVE having an equivalent weight of 1100, and was treated with an aqueous bath containing 11% KOH and 30% dimethylsulfoxide to hydrolyze the functional groups to carboxylate and sulfonate groups. The membrane was mounted with the carboxylate side toward the cathode. The electrodes were positioned so that there was a 3 mm gap between them. The cell was constructed so that a hydraulic head corresponding to approximately 25.4 cm (10 inches) of water on the cathode side pressed the membrane against the anode. The cell was operated at 90°C with a current density of 31 A/dm². A saturated solution of purified sodium chloride was fed to the anolyte chamber at such a rate as to maintain a concentration of 200 g/1 NaCl. Water was added to the catholyte chamber to maintain the concentration of caustic produced at 32 + 1%.

After 7 days, the cell was performing at 96% current efficiency and 3.17.volts. The performance remained unchanged after 110 days of operation.

### Comparative Example A

Example 6 was repeated except that the cathode was made from uncoated mild steel expanded mesh. After 7 days, the cell was operating at 96.4% current efficiency and 3.51 volts. This is 340 mV higher than the activated cathode of Example 6. Example 7 - Performance of a one-side coated cathode in a finite gap membrane cell.

Example 5 was repeated except that the coating was applied only to the one face of the cathode which faced the membrane in the cell. This cathode was then installed and operated in a test cell under the same conditions as Example 6.

After 7 days, the cell was operating at 97.6% current efficiency and 3.20 volts. After 30 days, the cell voltage was 3.18 volts and remained unchanged after 110 days of operation. This is 330 mV lower than the mild steel cathode of Comparative-Example A.

### Example 8 - Performance of a two-side coated cathode in a zero gap membrane cell.

A cathode prepared as per Example 5 was mounted in a small cell having an active area of ₄5 cm². The membrane comprised a 38 micron (1.5 mil) layer of TFE/EVE having an equivalent weight of 1080 and a 100 micron (4 mil) layer of TFE/PSEPVE having an equivalent weight of 1100, was coated on both sides with an inorganic nonconductive layer comprised of ZrO₂ particles bonded with a solution in ethanol of a 950 equivalent weight copolymer of TFE/PSEPVE and dried, and was treated with KOH as in Ex. 6 to hydrolyze the functional groups to carboxylate and sulfonate groups. A dimensionally stable anode was used and the electrodes were positioned close together with the membrane between them such that there was no gap between the membrane and either electrode.^{*} The membrane was mounted with the carboxylate side toward the cathode. The cell was operated at 90°C with a current density of 31 A/dm². A saturated solution of purified sodium chloride was fed to the anolyte chamber at such a rate as to maintain the concentration at 200 g/l NaCl. Water was added to the catholyte chamber to maintain the concentration of caustic produced at 32 + 1%.

After 7 days, the cell was performing at 97.8% current efficiency and 3.09 volts.

### Example 9 and Comparative Examples B, C and D

Samples of mild steel cathode screen made of 0.23 cm (0.092 inch) diameter wire spaced on 0.42 cm centers (6 mesh), cleaned by blasting with 700 micron (24 mesh) alumina grit at 5.5 x 10⁵ Pa (80 psi), were plasma sprayed at the following conditions:
Volts - 40
Amperes - 620
Power - 24.8 kw
TTWD (torch to workpiece d_istance) - . 6.3-7.6 cm (2.5 - 3 inches)
Arc gas - 2.63 m³/hr (93 CFH) argon at 3.45 x 10⁵ Pa (50 psi)

Four different nickel/aluminum alloy compositions were used, having nickel/aluminum weight ratios of 52/48 (Ex. B), 55/45 (Ex. C), 57/43 (Ex. 9) and 62/38 (Ex. D). All had particle sizes of 42-110 microns (140 to 325 mesh). The coating thickness applied was 152-178 microns (6-7 mils).

The plasma spray coated cathodes were activated by leaching successively in 2% aqueous caustic at 25°C, 5% aqueous caustic at 25°C, 10% aqueous caustic at 25°C, and 10% aqueous caustic at 80°C, each stage being carried out until hydrogen evolution ceased before proceeding to the next stage.

Each cathode (circular disk, 8.25 cm or 3.25 inches in diameter) was tested for performance in a small chloralkali cell as follows. The cell had anode and cathode compartments separated by a membrane of a perfluorinated ion exchange polymer having sulfonate groups; the area of membrane in use was circular, 3.5 cm in diameter. The anode was a platinum screen. A reference standard calomel electrode and the cathode to be tested were placed in the cathode compartment, with the calomel electrode as close as possible to, or in contact with, the cathode under test. The anode compartment was filled with a sodium chloride solution (250g NaCl/liter of solution); the cathode compartment was filled with a sodium chloride/sodium hydroxide solution containing about 13% sodium hydroxide (3 liters of the above NaCl solution, 1.5 liters water and 585g NaOH). Electrolysis was carried out at a current density of 15.5 A/dm at ca. 90°C, until stable electrode potentials were attained. The difference in potential between the test cathode and reference calomel electrode was measured with a high impedance digital voltmeter at intervals throughout the electrolysis period. The performance was compared against an uncoated mild steel cathode, and the results given below are reported as the millivolts advantage for the coated cathode vs. mild steel.

Each test cathode was then subjected to a sequence of water spray at 1.03 x 10 Pa (1500 psi) for 3 minutes on each side of the cathode to simulate the conditions of removal of a spent asbestos diaphragm and baking at 355°C for 4 hours to simulate the baking a newly applied asbestos diaphragm, even though no asbestos was actually removed or deposited. The amount of Raney nickel coating which spalled off during the water spraying was collected by filtration and weighed. The cell performance of the washed and baked cathode was again evaluated. This sequence was carried out ten times for each test cathode. The results are summarized in Tables I and II..

Table II

### INDUSTRIAL APPLICABILITY

The present invention is useful whenever Raney nickel coated electrodes are desired. It finds use especially in the chloralkali field where low hydrogen overvoltage cathodes are needed. The cathodes are more durable than those of the prior art, and have other advantages set forth above.

## Claims

1. A process for making a low-hydrogen-overvoltage cathode of the Raney nickel type for use in a chloralkali,cell, which process is characterised by
(a) plasma spraying a coating of a nickel/ aluminum alloy composition containing 56 to 59% by wt. nickel onto a foraminous substrate of iron, ferrous alloy, nickel or nickel alloy, and
(b) leaching aluminum from said coating by contacting the article prepared in step (a) with a caustic solution.

2. A process according to claim 1 wherein said nickel/aluminum alloy composition used in step (a) is in the form of 36 to 90 µm particles.

3. A process according to claim 2 wherein said nickel/aluminum alloy composition used in step (a) is in the form of 36 to 53 pm particles.

4. A process according to claim 1, 2 or 3 wherein the coating made in step (a) is 13 to 508 pm thick.

5. A process according to claim 4 wherein the coating made in step (a) is 127 to 254 pm thick.

6. A process according to any one of the preceding claims wherein said plasma spraying is carried out with an argon or nitrogen gas plasma generated with 20 to 30 kilowatts of power.

7. A process according to any one of the preceding claims wherein said step (b) is carried out for a time sufficient to remove 70 to 90% by weight of the aluminum from said coating.

8. A process according to any one of the preceding claims wherein said caustic solution used in step (b) is 5 to 15% by weight aqueous NaOH, and said contacting is for a time of 5 hours to 1 day.

9. A process according to any one of the preceding claim_{'}s wherein said nickel/aluminum alloy composition contains 56.5 to 57.5% by wt. nickel.

10. A process according to claim 9 wherein said nickel/aluminum alloy composition is substantially 57% by wt. nickel.

11. A chloralkali cell comprising a cathode compartment, a cathode disposed within said cathode compartment, an anode compartment, an anode disposed within said anode compartment and a separator disposed between said anode and cathode compartments, wherein said cathode has been made by a process as claimed in any one of the preceding claims.

12. A chloralkali cell according to claim 11 wherein said separator is a liquid permeable diaphragm.

13. A chloralkali cell according to claim 12 wherein said diaphragm comprises asbestos fibers.

14. A chloralkali cell according to claim 11 wherein said separator is a membrane of highly fluorinated ion-exchange polymer.

15. A process for electrolysis of an alkali metal chloride in an electrochemical cell divided into anode and cathode compartments by a separator, wherein an aqueous alkali metal chloride solution is introduced into the anode compartment of said cell, an electric current is passed through said cell, and aqueous alkali metal hydroxide solution is removed from said cathode compartment and chlorine is removed from said anode compartment, wherein said electrochemical cell is a chloralkali cell as claimed in any one of claims 11 to 14.
